

Sept. 13, 1960

W. L. DIEHL ET AL

2,952,568

CONTINUOUS HOT DIP GALVANIZING OF METAL STRIP

Original Filed Aug. 19, 1955



INVENTORS

William L. Diehl &  
Henry S. Bell

*Hooper, Leonard & Quell  
Their Attorneys*

1

2,952,568

## CONTINUOUS HOT DIP GALVANIZING OF METAL STRIP

William L. Diehl, St. Clairsville, Ohio, and Henry S. Bell, Wheeling, W. Va., assignors to Wheeling Steel Corporation, Wheeling, W. Va., a corporation of Delaware

Original application Aug. 19, 1955, Ser. No. 529,562, now Patent No. 2,875,096, dated Feb. 24, 1959. Divided and this application Mar. 26, 1958, Ser. No. 724,144.

### 1 Claim. (Cl. 117—102)

This invention relates to the continuous hot dip galvanizing of metal strip and more particularly to an improved process which contributes importantly to the ability to produce galvanized strip of optimum quality at unprecedented speed. This application is a division of our co-pending application Serial No. 529,562, filed August 19, 1955, now Patent No. 2,875,096.

As continuous line speeds have increased during the past decade or so great difficulty has been experienced in producing by continuous hot dip galvanizing galvanized strip of uniform optimum quality. The increased speed of the strip produces a strong tendency of the strip to carry with it an excessive quantity of spelter as the strip emerges from the bath of molten spelter and there is also a tendency for the coating on the galvanized strip to be relatively thick near the edges of the strip and relatively thin near the center of the strip.

It is possible by the use of grooved exit or coating rolls to counteract to some extent the above mentioned tendencies, but for the higher speeds which are now commercial grooved exit rolls do not adequately serve the purpose. Moreover, while for some intermediate speeds grooved exit rolls might be designed which would produce galvanized strip of optimum quality for a particular strip speed in the application of a particular weight of coating to a strip of a particular gauge, such rolls would not be satisfactory if the conditions should be substantially changed.

We have found that the tendency of the strip to carry an excessive amount of molten spelter up out of the bath when the strip speed increases can be counteracted or compensated for by regulating the drive of the exit rolls so that the exit rolls inhibit the movement of spelter upwardly between the rolls relatively to the effect of the exit rolls upon upward movement of the spelter when the exit rolls are normally driven. We reduce the speed at which the exit rolls are driven. The speed at which the exit rolls should be driven depends upon the speed and gauge of the strip and the thickness of coating desired. Generally speaking, the faster the speed of the strip and the thinner the coating desired the greater should be the difference between the speed of the strip and the speed of the exit rolls. The exit rolls should be driven at a speed somewhat slower than the speed of the strip.

Another factor which causes difficulty is the capillary attraction of the strip for the spelter. The exit rolls will break down the capillary attraction to a certain extent but their ability to do so is lessened as the strip speed and coating thickness increase. We have found it highly desirable to provide means engaging the strip in the molten spelter bath before the strip reaches the exit rolls to inhibit the tendency of spelter to cling to the strip, or, in other words, to break down the capillary attraction of the strip for the spelter. We desirably bring rolls to bear against the respective faces of the strip in the bath before the strip reaches the exit rolls.

2

The means engaging the strip in the bath before the strip reaches the exit rolls to inhibit the tendency of spelter to cling to the strip should be so positioned relatively to the exit rolls that substantial capillary attraction of the spelter to the strip cannot be set up between said means and the exit rolls.

If such means are spaced too far away from the exit rolls capillary attraction between the strip and the spelter may be set up all over again before the strip reaches the exit rolls even though it has been reduced by such means. We prefer to employ opposed rolls in the bath arranged to bear against the respective faces of the strip before the strip reaches the exit rolls and thereby inhibiting the tendency of spelter to cling by capillary attraction to the strip, such opposed rolls being so positioned relatively to the exit rolls that substantial capillary attraction of the spelter to the strip cannot be set up between such rolls and the exit rolls. The capillarity reducing rolls desirably have faces resistant to wetting by molten spelter. Such rolls may be made of stainless steel or they may be chromium plated or surfaced with some hard, glassy material resistant to wetting by molten spelter. Materials which are resistant to wetting by molten spelter are known to those skilled in the art.

The capillarity reducing rolls are preferably relatively resiliently urged toward the strip. One of those rolls may be mounted for rotation about a fixed axis and the other may be resiliently pressed toward the roll which is mounted for rotation about a fixed axis.

The distance between the capillarity reducing rolls and the exit or coating rolls depends upon the speed of the strip, the gauge of the strip and the thickness of the galvanized coating being applied to the strip. It is not possible to state empirically what that distance should be just as it is not possible to state empirically just what the speed of the exit rolls should be since the variables which have been mentioned have to be taken into consideration. However, a person skilled in the art following our teaching will have no difficulty ascertaining the optimum speed of the exit rolls and the optimum distance between the capillarity reducing rolls and the exit rolls for a particular strip speed coupled with a particular strip gauge and a particular thickness of coating.

Either grooved or ungrooved exit rolls may be used. For ungrooved rolls the speed differential between the rolls and the strip for high strip speeds may be somewhat less than when grooved rolls are employed.

The capillarity reducing rolls may be pressed together by any convenient means, the purpose being to press those rolls against the strip with sufficient pressure that as the strip advances it will cause the capillarity reducing rolls to turn by engagement with the strip. Thus normally the capillarity reducing rolls, being driven by the strip, turn at a peripheral speed substantially equal to the linear speed of the strip.

The capillarity reducing rolls are preferably of smaller diameter than the exit rolls. We have found that generally speaking it is desirable to have the capillarity reducing rolls not greater than about three inches in diameter. They are preferably ungrooved and as above stated preferably have faces resistant to wetting by molten spelter. For example, the capillarity reducing rolls may be made of, or at least faced with, alloy steel.

For very high speeds it may be desirable to provide capillarity reducing rolls in tandem, i.e., to provide more than one set of such rolls engaging the strip successively as the strip advances through the spelter bath toward the exit rolls.

Other details, objects and advantages of the invention will become apparent as the following description of a present preferred method of practicing the same proceeds.

In the accompanying drawing we have shown apparatus capable of use in practicing the invention, the figure being a fragmentary view partly in elevation and partly in vertical cross-section of a hot dip galvanizing pot.

We have found that when the exit rolls of a galvanizing pot are rotated so that their peripheral speed equals the linear speed of the strip being galvanized there is a critical speed range beyond which the coating cannot be effectively controlled either as to weight or as to quality due to the fact that the increased strip speed tends to carry an excess of molten spelter into the exit rolls, largely by capillarity, which excess spelter cannot be properly distributed over the exit rolls and the strip. At times streams of excess coating metal and imperfections occur on the coated strip and the longitudinal edges of the strip may be relatively heavily coated due to the excess of molten spelter carried up by the exit rolls. We have found that the critical speed above referred to is substantially in the range 140-160 feet per minute. The critical speed varies with the gauge of the strip being coated, the composition of the spelter bath, the fluidity of the bath, the temperature of the bath, the thickness of the coating being applied to the strip, etc.

Continuous galvanizing lines are now operated at speeds above 300 feet per minute and speeds in the range 500-600 feet per minute are probable in the near future. For strip speeds in excess of the critical range above referred to we drive the exit rolls at speeds different from the strip speed and/or provide for breaking the capillarity of the molten metal before the strip reaches the exit rolls to reduce the amount of molten spelter carried up by the strip.

When the strip speed is in excess of the above mentioned critical speed we prefer to operate the exit rolls at a peripheral speed in the range 30-60 feet per minute. All of the speeds mentioned are subject to variation depending upon the variations in operating conditions as referred to above.

Referring now more particularly to the drawing, there is shown a galvanizing pot designated generally by reference numeral 2 and which may be of conventional construction. It is adapted to contain molten spelter, the level of the molten spelter in the galvanizing pot 2 being indicated by the line 3. By "spelter" we mean any molten bath suitable for galvanizing and which is primarily zinc. The spelter may be substantially all zinc, or it may have other metals admixed with the zinc, such, for example, as aluminum, lead, antimony, cadmium, tin, and so on, either singly or in various combinations.

The exit rolls, sometimes called coating rolls, are shown at 4, being mounted in conventional manner partly immersed in the molten spelter and partly extending above the surface of the molten spelter. As shown in the drawing the surface of the molten spelter is substantially at the elevation of the axes of the exit rolls 4. The exit rolls are provided with driving means comprising intermeshing gears 14 driven by a driving gear 15 on a driving shaft 16.

The strip enters the galvanizing pot in conventional manner and passes through the molten spelter and about a guide roll 5 rotatably mounted below the surface of the spelter, the strip, which is designated by reference numeral 6, passing vertically upwardly from the guide roll 5 between the exit rolls 4 as shown.

We provide opposed capillarity reducing rolls 7 and 8 adapted to engage the strip at opposite faces thereof as shown in the drawing. The capillarity reducing rolls 7 and 8 have faces resistant to wetting by molten spelter

and are relatively resiliently urged toward the strip. In the form shown the roll 7 is mounted for rotation about a fixed axis and the roll 8 is resiliently pressed toward the roll 7. The roll 8 is rotatably mounted in a pivoted mounting structure 9 which is pivoted at 10 to a stationarily mounted bracket 11. Connected with the mounting structure 9 is an outwardly extending arm 12 carrying a weight 13 which is adjustably positionable along the arm. The structure 9, the arm 12 and the weight 13 are to all intents and purposes unitary and the weight may be adjusted along the arm as desired to resiliently press the roll 8 toward the roll 7 with the desired force. The rolls 7 and 8 are both freely rotatable and are turned by the movement of the strip in contact therewith.

The rolls 7 and 8 are so positioned relatively to the exit rolls 4 that substantial capillary attraction of the spelter to the strip cannot be set up between the rolls 7 and 8 and the rolls 4. The rolls 7 and 8 reduce or break the capillary attraction of the spelter for the strip and thus cooperate with the exit rolls 4 in controlling the application of the spelter to the strip.

As mentioned above, the distance between the rolls 4 and the rolls 7 and 8 cannot be empirically stated and depend upon the speed of the strip, the gauge of the strip and the thickness of the coating applied to the strip. However, by slowing down the speed of the rolls 4 relatively to the strip and maintaining the distance between the rolls 4 and the rolls 7 and 8 as above explained 30 galvanized strip of optimum quality can be produced at unprecedented speed.

While we have illustrated and described a present preferred method of practicing the invention it is to be distinctly understood that the invention is not limited thereto but may be otherwise practiced within the scope of the following claim.

We claim:

In the continuous hot dip galvanizing of metal strip in which the strip is delivered upwardly at high speed out of the galvanizing bath of molten spelter between exit rolls partly immersed in the bath engaging the respective faces of the strip and arranged with their axes parallel and generally horizontal and which exit rolls are normally driven with their portions next the strip moving upwardly, the step of inhibiting the carrying up out of the bath of an excessive amount of molten spelter which comprises positively driving the exit rolls in the direction of advance of the strip at a speed somewhat slower than the speed of the strip whereby the exit rolls exert a drag on the molten spelter uniformly across the strip and at the edges and thereby restrain movement of spelter upwardly between the rolls relatively to the effect of the exit rolls upon upward movement of the spelter when the exit rolls are driven at a speed equal to the speed of the strip.

#### References Cited in the file of this patent

#### UNITED STATES PATENTS

|    |           |              |               |
|----|-----------|--------------|---------------|
| 60 | 2,364,904 | Keller       | Dec. 12, 1944 |
|    | 2,377,632 | Keller       | June 5, 1945  |
|    | 2,401,374 | Sendzimir    | June 4, 1946  |
|    | 2,740,729 | Hodil        | Apr. 3, 1956  |
|    | 2,797,476 | Sendzimir    | July 2, 1957  |
| 65 | 2,875,096 | Diehl et al. | Feb. 24, 1959 |

#### OTHER REFERENCES

Bablic: Galvanizing (Hot Dip), page 434, 3rd ed., 1950; Spon Ltd., London.